



US006140753A

# United States Patent [19]

Joo et al.

[11] Patent Number: 6,140,753

[45] Date of Patent: Oct. 31, 2000

[54] CATHODE FOR AN ELECTRON GUN

96-15634 5/1996 Rep. of Korea .

[75] Inventors: **Gyu-Nam Joo; Jong-Seo Choi; Yoon-Chang Kim**, all of Suwon-shi, Rep. of KoreaPrimary Examiner—Ashok Patel  
Attorney, Agent, or Firm—Baker & McKenzie[73] Assignee: **Samsung Display Devices Co., Ltd.**,  
Rep. of Korea**ABSTRACT**

[21] Appl. No.: 09/063,943

[22] Filed: Apr. 21, 1998

**Foreign Application Priority Data**

Dec. 30, 1997 [KR] Rep. of Korea 97-97095

[51] Int. Cl.<sup>7</sup> H01J 1/20

[52] U.S. Cl. 313/346 R

[58] Field of Search 313/346 R, 346 DC,  
313/270, 337

The present invention includes a cathode for an electron gun having a base metal mainly composed of nickel and containing one kind of reducing element at least, a metal layer mainly composed of nickel or nickel-zirconium on the upper side of the base metal, and an electron emitting material layer containing alkaline earth metal oxide including barium at least on the upper side of the metal layer. The metal layer is formed by spreading nickel or nickel-zirconium on the base metal and heating it or by adhering nickel or nickel-zirconium powder thereon to have particle smaller than that of the base metal, to increase its life cycle under a high current density load by ensuring a diffusion route of reducing element steadily for good generation of free radical barium atom. In another aspect, the present invention proposes a cathode for an electron gun further having a second electron emitting material layer containing both of lanthanum compound and magnesium compound or lanthanum-magnesium mixed compound in alkaline earth metal oxide containing barium at least on the upper side of the electron emitting material layer.

**References Cited****U.S. PATENT DOCUMENTS**5,118,984 6/1992 Saito et al. 313/346 R  
5,592,043 1/1997 Gartner et al. 313/347 R X  
5,808,404 9/1998 Koizumi et al. 313/346 R**FOREIGN PATENT DOCUMENTS**

91-257735 9/1991 Japan .

**23 Claims, 7 Drawing Sheets**

Fig. 1



Fig.2



Fig.3



Fig.4



Fig.5



Fig.6



PRIOR ART

Fig.7



PRIOR ART

## CATHODE FOR AN ELECTRON GUN

## BACKGROUND OF THE INVENTION

## 1. Field of the Invention

The present invention relates to a cathode for an electron gun used in a cathode ray tube, and more particularly, it relates to a cathode for an electron gun for increasing its life cycle under a high current density load by ensuring a diffusion route of reducing element steadily, used for generating free radical barium atom.

## 2. Description of the Prior Art

A cathode ray tube is a device for forming an image by excitation light emission of a fluorescent material of a screen by landing an electron emitted from an electron gun and accelerated by high voltage on the fluorescent material.

FIG. 6 is a general structural diagram of a cathode for an electron gun in a cathode ray tube. In FIG. 6, the cathode comprises a heater 4 in a sleeve 2, a cap-formed base metal 6 mainly composed of nickel Ni and containing a small amount of reducing elements such as silicone Si and magnesium Mg on the upper side of sleeve 2, and an electron emitting material layer 8 mainly composed of alkaline earth metal oxide containing barium at least on the cap-formed base metal 6.

In such a cathode, the metal oxide and the reducing element react to each other by heat generated from the heater to generate free radical barium atom, and thereafter thermion is emitted by using free radical barium.

An electron emission capacity of the cathode for the electron gun is influenced by a supply amount of free radical barium contained in the metal oxide.

However, since the cathode ray tube has a tendency of enlargement and high precision recently, a cathode which can supply free radical barium atom for a long time in high current density is required.

In Korean patent laid-open No. 96-15634, a cathode restraining free radical barium atom from evaporating by adding both of lanthanum La compound and magnesium compound Mg or La—Mg mixed compound to the electron emitting material layer containing alkaline earth metal oxide is disclosed.

However, in the conventional cathode, an intermediate layer 10 is generated in a boundary between the base metal 6 and the electron emitting material layer 8 by reaction as shown in FIG. 7, and it results to shorten the life of the cathode under high current density load of 2~3 A/cm<sup>2</sup>.

The intermediate layer 10 is generated by reaction of barium oxide pyrolyzed from barium carbonate and silicone or magnesium.

## [Reaction formula 1]



## [Reaction formula 2]



Free radical barium atom generated by the reaction for formula 1 or 2 is served to emit electron, however, MgO or Ba<sub>2</sub>SiO<sub>4</sub> is additionally generated by the same reaction formulas to generate the intermediate layer 10 in the boundary between the base metal 6 and the electron emitting material layer 8.

Such an intermediate layer 10 interferes the reaction for generating free radical barium atom requiring the reducing

agent by obstructing diffusion of the reducing agent contained in the base metal 6, to shorten the life of the cathode. In addition, since the intermediate layer 10 has a high resistance, it limits the current density possible to emit the electron by interfering flow of the electron emitting current.

In another aspect, a cathode for an electron gun comprising a metal layer mainly composed of tungsten of which the reducing degree is same as or smaller than silicone or magnesium and larger than nickel between the base metal and the electron emitting material layer, and the electron emitting material layer containing rare earth metal oxide to decompose the compound generated from the reaction, and thereby enabling the reducing element in the metal layer to serve to generate free radical barium atom is disclosed in Japanese patent laid-open No. 91-257735.

However, the cathode described above is stable at the beginning but its life cycle is suddenly deteriorated with the lapse of time since the additional reaction compound is generated when free radical barium atom is generated.

## SUMMARY OF THE INVENTION

Accordingly, the present invention is directed to a cathode for an electron gun that substantially obviates one or more of the problems due to limitations and disadvantages of the related art.

An object of the present invention is to provide a cathode for an electron gun for increasing its life cycle under a high current density load by ensuring a diffusion route of reducing element of a base metal steadily, used for good generation of free radical barium atom.

Additional features and advantages of the invention will be set forth in the description which follows, and in part will be apparent from the description, or may be learned by practice of the invention.

The objectives and other advantages of the invention will be realized and attained by the structure particularly pointed out in the written description and claims hereof as well as the appended drawings.

To achieve these and other advantages and in accordance with the purpose of the present invention, as embodied and broadly described, there is disclosed a cathode for an electron gun comprising:

a base metal mainly composed of nickel and containing one kind of reducing element at least;  
a metal layer mainly composed of nickel or nickel-zirconium on the upper side of the base metal; and  
an electron emitting material layer containing alkaline earth metal oxide including barium at least on the upper side of the metal layer.

The metal layer is formed by spreading nickel or nickel-zirconium on the upper side of the base metal and heating it or by adhering nickel or nickel-zirconium powder thereon to have particle smaller than that of the base metal.

In another aspect, the present invention provides a cathode for an electron gun further comprising a second electron emitting material layer containing both of lanthanum compound and magnesium compound or lanthanum-magnesium mixed compound in alkaline earth metal oxide containing barium at least on the upper side of the electron emitting material layer.

According to the present invention, since the metal layer having particle smaller than that of the base metal effectively disperses the material generated by the reaction of BaO and Si or Mg to prevent the generation of the intermediate layer having high resistance and to ensure a diffusion route of the reducing element steadily, the reaction for generating free

radical barium atom requiring the reducing element can be continued to increase life cycle of the cathode under high current density load of 2~3 A/cm<sup>2</sup>.

It is to be understood that both the foregoing general description and the following detailed description are exemplary and explanatory and are intended to provide further explanation of the invention as claimed.

#### BRIEF DESCRIPTION OF THE DRAWINGS

The accompanying drawings, which are included to provide a further understanding of the present invention and are incorporated in and constitute a part of this specification, illustrate embodiments of the present invention and together with the description serve to explain the principles of the present invention:

In the drawings:

FIG. 1 is a sectional view of a cathode for an electron gun in accordance with one embodiment of the present invention;

FIG. 2 is an enlarged sectional view of a main part of a cathode for an electron gun in accordance with one embodiment of the present invention;

FIG. 3 is a diagram showing a life cycle characteristic of a cathode for an electron gun in accordance with one embodiment of the present invention;

FIG. 4 is a sectional view of a cathode for an electron gun in accordance with another embodiment of the present invention;

FIG. 5 is a diagram showing a life cycle characteristic of a cathode for an electron gun in accordance with another embodiment of the present invention;

FIG. 6 is a sectional view of a conventional cathode for an electron gun; and

FIG. 7 is an enlarged sectional view of a conventional cathode.

#### DESCRIPTION OF THE PREFERRED EMBODIMENTS

Reference will now be made in detail to the preferred embodiments of the present invention, examples of which are illustrated in the accompanying drawings. Like reference numerals denote like reference parts throughout the specification and drawings.

#### EMBODIMENT 1

As shown in FIG. 1, a cathode for an electron gun according to a first embodiment of the present invention comprises a cap-formed base metal 6 mainly composed of Ni and containing reducing elements such as Si and Mg on upper opening portion of a sleeve 2 in which a heater 4 is mounted.

The cathode for the electron gun further comprises a metal layer 12 containing pure Ni or Ni—Zr on the upper side of the base metal 6, and an electron emitting material layer 8 composed of alkaline earth metal oxide such as ternary carbonate (Ba.Sr.Ca)CO<sub>3</sub> or binary carbonate (Ba.Sr)CO<sub>3</sub> containing Ba at least on the upper side of the metal layer.

In the present embodiment, to disperse the material generated from the reaction of BaO and Si or Mg and accumulated in the boundary between the base metal 6 and the electron emitting material layer 8, a metal layer 12 composed of fine-grained pure Ni or Ni—Zr is formed in the boundary.

Since the metal layer 12 according to the present embodiment is formed of particles smaller than those of the base metal 6 as shown in FIG. 2, the diffusion route of the reducing element contained in the base metal 6 is dispersed, and therefore, the reaction of BaO and Si or Mg is performed in many area of the metal layer 12, the intermediate layer 10 is restrained from being accumulated, and the reducing element such as Si and Mg is smoothly diffused to be served to generate free radical barium atom.

In addition, since the metal layer 12 is formed of the same components as the base metal 6, i.e. pure Ni or Ni—Zr the intermediate layer is not generated from the reaction unlike the conventional metal layer coated with W.

The metal layer 12 is obtained by forming a layer of Ni or Ni—Zr to a thickness of 200~20,000 Å by sputtering, and heating it in the temperature of 700~1,100° C. in an inactive or vacuum condition to perform an alloying and diffusion between the base metal 6 and the metal layer 12.

The thickness of the metal layer 12 is preferably 200~20,000 Å.

It is difficult to ensure the diffusion route of the reducing element when the thickness is less than 200 Å and when the thickness is more than 20,000 Å, it interferes the diffusion of the reducing element.

The thickness of the metal layer 12 of the present embodiment is 3000~10,000 Å the optimum.

The metal layer 12 is formed by adhering Ni or Ni—Zr powder on the upper side of the base metal 6.

At this point, the adhesion is realized by physical, chemical, or mechanical methods such as spray, print, electrodeposition, or metallic salt solution.

The electron emitting material layer of ternary carbonate or binary carbonate is formed on the upper side of the metal layer 12 to the thickness of 20~80 μm by spray. At this point, the thickness of the entire cathode must not exceed 200 μm.

#### EMBODIMENT 2

A second embodiment of the present invention proposes a cathode for an electron gun comprising a second electron emitting material layer instead of the electron emitting material layer of the first embodiment.

As shown in FIG. 1, the second electron emitting material layer 80 is formed on the upper side of the metal layer 12 composed of pure Ni or Ni—Zr by adding both of La compound and Mg compound or La—Mg mixed compound in alkaline earth metal oxide such as ternary carbonate (Ba.Sr.Ca)CO<sub>3</sub> or binary carbonate (Ba.Sr)CO<sub>3</sub> containing Ba at least.

The La compound and Mg compound or La—Mg mixed compound restrains evaporation of free radical Ba atom to be continuously supplied. The weight of the La compound and Mg compound or La—Mg mixed compound is preferably 0.01~1 weight % of the carbonate.

When the weight thereof is less than 0.01 weight %, the evaporation of free radical Ba atom can not be effectively restrained and when the weight thereof is more than 1 weight %, the electron emitting capacity at the beginning can be deteriorated.

According to the present embodiment, the intermediate layer 10 is effectively dispersed by the metal layer 12 and the evaporation of free radical Ba atom generated from the reaction of BaO and Si or Mg is restrained by the second electron emitting material layer 80.

The metal layer 12 according to the present embodiment is obtained by spreading Ni or Ni—Zr to a thickness of

200~20,000 Å on the upper side of the base metal **6**, and heating it in an inactive or vacuum condition to perform an alloying and diffusion between the base metal **6** and the metal layer **12**. Further, the metal layer **12** can be formed by adhering Ni or Ni—Zr powder on the upper side of the base metal **6**.

The second electron emitting material layer **80** composed of ternary carbonate or binary carbonate and further comprising both La compound and Mg compound or La—Mg mixed compound is formed on the upper side of the metal layer **12** to the thickness of 20~80 µm by spray coating.

At this point, the thickness of the entire cathode must not exceed 200 µm.

FIG. 3 shows a result of testing the life cycle characteristic of the cathode for the electron gun according to the present embodiment.

In FIG. 3, A shows the life cycle of the cathode according to the present embodiment comprising carbonate containing 0.5 weight % of La—Mg compound and the metal layer **12** having thickness of 3,000~5,000 Å.

B shows the cathode comprising carbonate containing 0.5 weight % of La—Mg compound and not having the metal layer **12**, and C shows the conventional cathode.

The test of life cycle is performed by measuring the decreasing amount of the electron emitting current while continuously operating for 6,000 hours.

At this moment, 2,000~3,000 µA of current is applied to each cathode.

As shown in FIG. 3, the cathode for the electron gun according to the present embodiment is considerably improved in its life cycle in high current in comparison with B or C according to the conventional art.

Using the cathode according to the present invention, 90% of first current value is maintained after operating for 6,000 hours in high current density.

### EMBODIMENT 3

As shown in FIG. 4, a cathode for an electron gun according to a third embodiment of the present invention comprises a base metal **6**, a metal layer **12** composed of pure Ni or Ni—Zr on the upper side of the base metal **6**, an electron emitting material layer **8** composed of ternary carbonate or binary carbonate containing Ba at least on the upper side of the metal layer **12**, and a second electron emitting material layer **80** composed of ternary carbonate or binary carbonate containing Ba at least and further containing both of La compound and Mg compound or La—Mg mixed compound on the upper side of the electron emitting material layer **8**.

According to the second embodiment, free radical Ba atom may be excessively evaporated since the reducing element composed of Ni or Ni—Zr and the reducing element contained in the base metal **6** urge the reduction of free radical Ba atom.

Accordingly, in the present embodiment, to disperse the material generated from the reaction of BaO pyrolyzed from carbonate and Si or Mg and accumulated in the boundary between the base metal **6** and the electron emitting material layer **8**, the metal layer **12** containing pure Ni or Ni—Zr is formed therebetween.

In addition, to restrain the evaporation of free radical Ba atom in the electron emitting material layer **8**, the second electron emitting material layer **80** composed of carbonate containing 0.01~1 weight % of La compound and Mg compound or La—Mg mixed compound is formed.

The metal layer **12** is obtained by spreading Ni or Ni—Zr to a thickness of 200~20,000 Å on the upper side of the base metal **6**, and heating it in an inactive or vacuum condition to perform an alloying and diffusion between the base metal **6** and the metal layer **12**.

The thickness of the metal layer **12** is preferably 200~2000 Å, considering the thickness of the electron emitting material layer **8** and the second electron emitting material layer **80** formed on the upper side of the metal layer **12**.

The thickness of the metal layer **12** of the present embodiment is 400~1,200 Å the optimum.

In addition, the metal layer **12** can be formed by adhering Ni or Ni—Zr powder on the upper side of the base metal **6**.

On the upper side of the metal layer **12** formed as described above, the electron emitting material layer **8** composed of ternary carbonate or binary carbonate is coated to the thickness of 20~80 µm, and on the upper side of the electron emitting material layer **8**, the second electron emitting material layer **80** composed of ternary carbonate or binary carbonate and further containing both of La compound and Mg compound or La—Mg mixed compound is coated to the thickness of 20~80 µm in order to manufacture the cathode of the entire thickness does not exceed 200 µm.

FIG. 5 shows a result of testing the life cycle characteristic of the cathode for the electron gun according to the present embodiment.

In FIG. 5, D shows the life cycle of the cathode according to the present embodiment comprising the metal layer **12** of which the thickness is 400~1,200 Å, the electron emitting material layer **8** on the upper side of the metal layer **12**, and the second electron emitting material layer **80** composed of carbonate containing 0.5 weight % of La—Mg compound. E shows the conventional cathode.

The test of life cycle is performed by measuring the decreasing amount of the electron emitting current while continuously operating for 6,000 hours. At this moment, 2,000~3,000 µA of current is applied to each cathode.

As shown in FIG. 5, the cathode for the electron gun according to the present embodiment is considerably improved in its life cycle in high current in comparison with the conventional art.

Using the cathode according to the present invention, 95% of first current value is maintained after operating for 6,000 hours in high current density.

In addition, according to the present embodiment, the maximum cathode current increases with the lapse of time.

According to the present invention, since the metal layer having fine grain formed between the base metal containing the reducing element and the electron emitting material layer composed of carbonate disperses the intermediate layer generated when generating free radical Ba atom to ensure the diffusion route of the reducing element steadily, free radical Ba atom can be continuously emitted.

In addition, since the inventive cathode comprises the electron emitting material layer containing both of La compound and Mg compound or La—Mg mixed compound, or further comprises the second electron emitting material layer containing both of La compound and Mg compound or La—Mg mixed compound, the evaporation of free radical Ba atom can be restrained.

As described above, since free radical Ba atom is continuously emitted and restrained to be evaporated due to the interaction of the metal layer and the electron emitting material layer or the second electron emitting material layer,

the life cycle is improved even under high current density load of 2~3 A/cm<sup>2</sup>.

In addition, the inventive cathode can be manufactured easily and at low price in comparison with the conventional impregnation cathode.

It will be apparent to those skilled in the art that various modifications and variations can be made in the cathode for the electron gun of the present invention without departing from the spirit or scope of the invention.

Thus, it is intended that the present invention cover the modifications and variations of this invention provided they come within the scope of the appended claims and their equivalents.

What is claimed is:

1. A cathode for an electron gun comprising:  
a base metal mainly composed of nickel and containing one kind of reducing element at least;  
a metal layer mainly composed of fine grained nickel and disposed on the upper side of said base metal; and  
an electron emitting material layer containing alkaline earth metal oxide including barium at least disposed on the upper side of said metal layer.

2. A cathode for an electron gun according to claim 1, wherein said metal layer is composed of nickel or nickel-zirconium.

3. A cathode for an electron gun according to claim 1 or 2, wherein said metal layer includes an alloying and diffusion layer adjacent the base metal.

4. A cathode for an electron gun according to claim 3, wherein said metal layer is formed of particles smaller than those of the base metal.

5. A cathode for an electron gun according to claim 1 or 2, wherein said metal layer comprises a layer of nickel or nickel-zirconium powder adhered on the upper side of the base metal.

6. A cathode for an electron gun according to claim 5, wherein said metal layer is formed of particles smaller than those of the base metal.

7. A cathode for an electron gun according to claim 1, wherein said metal layer has thickness of 200~20,000 Å.

8. A cathode for an electron gun according to claim 1, wherein said electron emitting material layer further containing both of lanthanum compound and magnesium compound or lanthanum-magnesium mixed compound.

9. A cathode for an electron gun according to claim 8, wherein said metal layer is composed of nickel or nickel-zirconium.

10. A cathode for an electron gun according to claim 8 or 9, wherein said metal layer includes an alloying and diffusion layer adjacent the base metal.

11. A cathode for an electron gun according to claim 10, wherein said metal layer is formed of particles smaller than those of the base metal.

12. A cathode for an electron gun according to claim 8 or 9, wherein said metal layer is nickel or nickel-zirconium powder.

13. A cathode for an electron gun according to claim 12, wherein said metal layer is formed of particles smaller than those of the base metal.

14. A cathode for an electron gun according to claim 8, wherein said metal layer has thickness of 200~20,000 Å.

15. A cathode for an electron gun according to claim 10 further comprising a second electron emitting material layer including both of lanthanum compound and magnesium compound or lanthanum-magnesium mixed compound in alkaline earth metal oxide containing barium at least on the upper side of said second electron emitting material layer.

16. A cathode for an electron gun according to claim 15, wherein said metal layer is composed of nickel or nickel-zirconium.

17. A cathode for an electron gun according to claim 15 or 16, wherein said metal layer is formed by spreading nickel or nickel-zirconium on the base metal and heating it.

18. A cathode for an electron gun according to claim 17, wherein said metal layer is formed of particles smaller than those of the base metal.

19. A cathode for an electron gun according to claim 15 or 16, wherein said metal layer is formed by adhering nickel or nickel-zirconium powder on the upper side of the base metal.

20. A cathode for an electron gun according to claim 19, wherein said metal layer is formed of particles smaller than those of the base metal.

21. A cathode for an electron gun according to claim 15, wherein said metal layer has thickness of 200~2000 Å.

22. A cathode for an electron gun comprising:  
a base metal mainly composed of nickel and containing one kind of reducing element at least;  
a metal layer consisting of fine grained nickel and disposed on the upper side of said base metal; and  
an electron emitting material layer containing alkaline earth metal oxide including barium at least disposed on the upper side of said metal layer.

23. A cathode for an electron gun comprising:  
a base metal mainly composed of nickel and containing one kind of reducing element at least;  
a metal layer consisting of fine grained nickel-zirconium and disposed on the upper side of said base metal; and  
an electron emitting material layer containing alkaline earth metal oxide including barium at least disposed on the upper side of said metal layer.

\* \* \* \* \*